

## UNITED STATES PATENT OFFICE

2,492,561

PACKING COMPOSITION FOR REMOVAL OF  
ZINC FROM ZINC-COATED ARTICLESHarry A. Eckman, Chicago, Ill., assignor to Crane  
Co., Chicago, Ill., a corporation of IllinoisNo Drawing. Application May 18, 1946,  
Serial No. 670,831

2 Claims. (Cl. 75—63)

1

This invention relates to a heat treatment process and more particularly is concerned with the object for removing zinc as a coating from zinc coated materials.

The invention is specially concerned with a method for accomplishing such object and avoiding all the undesirable effects resultant from the use of treatments heretofore employed.

A further important object is to provide for a method for removing zinc as a coating by the employment of a simple combined packing and treatment method using containers.

A further object is to eliminate the undesirable effect of zinc fumes experienced in previous methods employed in which the zinc fumes were found objectionable.

In order to obtain a better appreciation of the significance of this contribution it should be realized at the outset that zinc coated products, particularly those which are hot galvanized and machined are frequently found unsuitable for commercial use because of the subsequent discovery of a defective or non-uniform coating. It should be further understood that such articles however, can be used later as a non-coated product if the zinc coating can be satisfactorily removed from the surface of such article, as for instance, the removal of the zinc generally has been done by dissolving the zinc coating in an acid solution. However, this procedure has been costly and the surfaces of the material treated often are objectionably attacked by the acid, realizing that the acid in many instances penetrates into fissures or cracks and pin-holes frequently of very small size on the surface and then later resulting in surface corrosion.

One of the more important advantages obtained by the use of this invention is the elimination of all of the undesirable effects of the acid treatment of material.

Primarily it consists of heating the zinc coated articles, such as pipe fittings from which the coat is to be removed, to a temperature not to exceed approximately 1700° F. and affecting oxidation of the zinc without materially or appreciably changing the physical properties of the article itself. Preferably it has been found that the heating required should be done in containers, such as pots or the like.

2

It is important to realize however, that unless special care is taken during the course of the heat treatment, the zinc fumes formed will attack the uncoated areas, such as machine surfaces, threads and the like, and after subsequent oxidation, it results in a zinc oxide deposit adhering to such surfaces which is of course objectionable particularly in the case of parts finished to a specific machine tolerance, as for example pipe threads or other finished surfaces in which the matter of a relatively close fit is important.

It has been discovered that by packing the zinc coated articles to be treated in a suitable metallic material of desired fineness the usual detrimental effect of the volatilizing zinc in the way of zinc fumes is eliminated. It has been observed that the zinc fumes formed react with the surface of the metallic particles constituting the packed material and thereby forming alloys of zinc; thus the metallic packing material present in this manner functions as a fixing agent for the volatilizing zinc and the alloys of zinc thus formed are later broken down by oxidation.

It will be apparent to those skilled in the art that zinc coatings obtained by hot dipping consist of an outer layer of substantially pure zinc and an inner layer which is relatively thin and is alloyed to the iron surfaces. It will be further understood that the zinc in the outer layer of such coating volatilizes readily when heated at relatively low temperatures, while the alloy layer beneath is more stable and is eliminated upon subsequent oxidation.

It has been found that zinc coated products such as pipe fittings for example, treated in accordance with the procedure hereinafter described in greater detail shows substantially no zinc present on the surface even when tested with a chemical reagent such as a copper sulphate solution; and a further and more important benefit obtained is shown in the fact that machined or uncoated surfaces remain clean and unaffected. The latter is a very significant benefit derived.

As to the packing material employed, it may be any metal or metallic alloy having a melting point exceeding the temperature used in the course of heating and which is capable of reacting with the

volatilizing zinc. Ferrous materials, however, have been found most desirable. A typical mixture found acceptable is one consisting of twenty-five percent (25%) to seventy-five percent (75%) iron particles as essential components, carbonates up to ten percent (10%), and an amount of solid carbonaceous material not to exceed ten percent (10%) and the balance consisting of an inert refractory such as sand or clay.

It is preferable that the principal constituents of the packing material constitutes finely divided particles thus securing a large surface area for the reaction with volatilizing zinc fumes; the particle size however, should at the same time be large enough to allow free passage of gases and fumes. Comparatively coarse materials, such as cast iron chips, however, have been used successfully. Other readily available ferrous materials, such as grinding dust have also proven satisfactory.

For the best performance it has been found desirable to mix the metallic packing with a certain amount of inert or refractory substance, such as clay, kaolin, or sand to prevent the metal particles from sticking together after the heat treatment. More specifically coarse sand has been found most suitable and it may be present in amounts up to 75% of the compounded mixture.

It should be understood that the removal of the zinc covering depends upon the oxidation of the zinc by carbon dioxide ( $CO_2$ ). To insure this reaction it has been found desirable to add a certain amount of carbonaceous matter, such as powdered sea coal or charcoal, to the mixture. The carbon present provides for a certain reducing atmosphere consisting principally of carbon monoxide and it will be readily apparent to those skilled in the art that carbon monoxide at a temperature exceeding approximately  $1150^{\circ} F.$  exerts a carburizing effect on ferrous materials. Such carburizing effect at this temperature is slow and limited to a surface effect due to the slow diffusion of the iron carbides formed. With an increase in temperature, the carburizing action of carbon monoxide becomes increasingly rapid. It is desirable under this condition that the metallic packing component in the mixture should respond to carburization and this reaction is facilitated by the large surface of the relatively finely divided metallic particles in the mixture. Small amounts of zinc present on the surface of these particles do not affect the carburization. Metallic carbonates present in the mixture further exert a catalyzing effect energizing the carburizing reaction. As a result of the carburizing action of carbon monoxide, carbon dioxide is evidenced by the following formula:



The carbon dioxide thus resulting serves as an oxidizing agent for the zinc as illustrated by the following reaction:



It will be readily apparent that the above reactions mentioned are vitally important in effecting the oxidation of the zinc. By summarizing the above two reactions into one, the process can be expressed as below:



In order to facilitate the oxidation of the zinc it has been found desirable to incorporate a certain amount of a suitable carbonate in the pack-

ing mixture and the amount of carbonate added should preferably be in proportion to the carbon content of the packing compound so that the atmosphere within the packing mixture is maintained reducing. Too high carbon dioxide content will exert undesirable oxidizing effect of the ferrous material treated. Carbonates used in the mixture may be any carbonate suitable to generate carbon dioxide during the process of heating, such as calcium carbonate, magnesium carbonate, sodium carbonate, barium carbonate and the like. It has also been found that mixtures of the carbonate may be used to advantage depending upon the processing temperatures used. Satisfactory results have also been obtained without the addition of carbonate to the mixture. Under this condition, however, the procedure is relatively slower and less efficient.

As the carburizing action of carbon monoxide is rapidly increased with the corresponding increase in temperature insofar as the heating is concerned, the oxidation of the zinc similarly proceeds proportionately faster as the higher temperatures are attained. Metallic carbonates present facilitate further the carburizing reaction.

Material treated, such as cast iron, is limited to a relatively low maximum processing temperature in order to preserve the properties of the iron. However, malleable iron may be processed at temperatures in the vicinity of  $1600^{\circ} F.$  without any appreciable change in its property and this has been confirmed by tabulated comparative physical properties obtained on test bars poured from the same iron.

Insignificant amounts of zinc may be detected by chemical analysis on the outer surface of the processed articles and the amounts are so small as to be truly insignificant and can be regarded as impurity insofar as the effect upon the metal surface is concerned.

In summarizing the benefits of this process, it has been found possible to salvage hot galvanized pipe fittings for example, heretofore not suitable for commercial use due to the defective zinc coating but by removing the zinc coating these fittings have been salvaged and subsequently sold as "black" fittings, so termed by the trade.

It should of course be quite apparent that the detailed analysis with respect to the various elements above recited is only average or illustrative and it may vary accordingly. Therefore the scope of the invention should be measured by the following claims in relation to the prior art, as herein appended.

I claim:

1. A packing material suitable for the removal of the element zinc from machined zinc-coated articles whereby the latter are treated by heating said articles predeterminedly while packed in said packing material, the packing consisting of 25 to 75% iron particles as essential components, carbonates up to 10%, an amount of solid carbonaceous material not to exceed 10% and the balance an inert refractory material from the group consisting of sand and clay.

2. A packing material for the removal of the element zinc from machined zinc-coated articles by heating said articles while packed in said packing material to a temperature low enough not to exert any detrimental effect on the articles but high enough to effect desired removal of the zinc, the said packing material consisting of iron particles not to exceed 75% as essential components, carbonates up to 10%, an amount of solid car-

bonaceous fuel material approximating 10% and the balance an inert refractory material such as sand and clay.

HARRY A. ECKMAN.

REFERENCES CITED

The following references are of record in the file of this patent:

UNITED STATES PATENTS

| Number | Name  | Date         |
|--------|-------|--------------|
| 66,310 | Dodds | July 2, 1867 |

| Number      |
|-------------|
| 360,732     |
| 499,018     |
| 702,764     |
| 5 1,061,447 |
| 1,202,886   |
| 2,287,227   |

| 10 Number |
|-----------|
| 14,462    |

| Name        | Date          |
|-------------|---------------|
| Sawyer      | Apr. 5, 1887  |
| Frey        | June 6, 1893  |
| Babe et al. | June 17, 1902 |
| Burkey      | May 13, 1913  |
| Phelps      | Oct. 31, 1916 |
| Bowsher     | June 23, 1942 |

FOREIGN PATENTS

| Country       | Date           |
|---------------|----------------|
| Great Britain | Sept. 13, 1889 |